

July 4, 1939.

W. H. WOOD ET AL

2,164,850

METHOD OF CONDITIONING CHROME ALLOY WIRE AND APPARATUS  
FOR THE PRACTICE OF SAID METHOD  
Filed March 10, 1936



INVENTOR.  
William H. Wood  
and Oscar C. Trautman  
BY  
Fay, Oberlin & Fay  
ATTORNEYS.

## UNITED STATES PATENT OFFICE

2,164,850

METHOD OF CONDITIONING CHROME  
ALLOY WIRE AND APPARATUS FOR THE  
PRACTICE OF SAID METHODWilliam H. Wood, South Euclid, and Oscar C.  
Trautman, Parma, Ohio, assignors to Ira  
Crouse, Conneaut, Ohio

Application March 10, 1936, Serial No. 68,088

7 Claims. (Cl. 148—4)

Our invention pertains to improvements in the conditioning of wire and similar articles made of an alloy, such as nichrome and chrome alloys of iron, containing a high percentage of chromium. 5 As is well understood, many such alloys are annealed when quickly quenched from a temperature of about 2100° F. An object of our invention is the production of an article fully annealed and pickled as a continuous operation. We have invented a new method of securing these desired results in a continuous operation and apparatus 10 for the practice of said method.

To the accomplishment of the foregoing and related ends, said invention, then, consists of the means and steps hereinafter fully described and particularly pointed out in the claims; the annexed drawing and the following description setting forth in detail certain means and one mode of carrying out the invention, such disclosed 20 means and mode illustrating, however, but one of the various ways in which the principle of the invention may be used.

In said annexed drawing:

We have shown diagrammatically the elements 25 of the conditioning apparatus which we use, disclosing the essential relation therebetween for the practice of our novel method.

In the practice of our method, the material to be treated is heated by passing a suitable electric 30 current therethrough as the material is advanced past two electrodes in contact therewith. A current of 65 volts A. C. may be successfully used. For the advanced electrode we use a bath of metal, or alloy having a low melting point, which 35 bath also functions as a medium to effect the desired quenching of the material. An alloy of tin and lead having a melting point of 400° F. is suggested.

From the quenching bath the material is passed 40 quickly to a pickling bath and is passed therefrom quickly to a rinse bath, which preferably contains in solution an agent which will neutralize any of the pickling solution carried over.

To effect the desired pickling action a direct 45 current of electricity is passed between the material and an anode placed in the pickling bath, which anode is connected to one terminal of a source of electro-motive force. A current of from 6 to 10 volts may be used to secure the desired 50 electrolytic action.

Successful pickling demands an even distribution 55 of the electrolytic action throughout the wire in the bath. To secure such even distribution we connect the other terminal of the source of electro-motive force with both the quenching

bath and the rinsing bath, thereby securing a current flow from the source of electro-motive force to the material being treated and thence through said material. From the material the current will pass through the pickling bath to the anode therein which, as stated, is connected to the other terminal of said source of electro-motive force. The distribution of current flow between the material and the anode will be substantially uniform with a resultant uniformity of pickling 10 effect.

Referring to the drawing, our apparatus for the practice of said disclosed method comprises a rotating electrode 2 in contact with a wire 1 which is to be treated. This electrode 2 is connected to one terminal of a source of electro-motive force 3, the other terminal of which is electrically connected with the liquid metal in a quenching bath 4. The wire 1 is advanced into the liquid metal of the quenching bath 4, thereby completing a 20 circuit for the flow of current from the source 3. The wire is held beneath the liquid metal by rollers 5, and is guided out of the bath by an idling roller 6, over which it passes into a pickling bath 7, within which it is held by idling rollers 25 8. From the pickling bath 7 the wire is guided by the idling roller 9 over which it passes into the rinsing bath 10, within which it is held by the idling roller 11.

Within the pickling bath 7 the anode 12 is 30 placed in parallel relation with a substantial portion of the wire 1 therewithin. This anode is electrically connected with the positive terminal of a source 13 of direct current. The other terminal of said source 13 is connected electrically 35 with the quenching bath 4 and with the rinsing bath 10. It will readily appear that current from the source 13 will flow to the baths 4 and 10, from thence through that portion of the wire 1 which is therebetween, and from the said wire 1 40 through the solution of the pickling bath 7 to the anode 12, from which it travels to the other terminal of the source 13.

In operation, a wire 1 will be heated to a proper temperature, say in the neighborhood of 45 2100° F. by its resistance to the passage of an E. M. F. such as a 65 volt alternating current therethrough as it travels from the rotating electrode 2 to the quenching bath 4. It will be understood that the wire 1 is drawn through the 50 apparatus by suitable means not shown, at a speed so proportioned to the current strength between electrode 2 and quenching bath 4, that the wire will have the desired temperature as it enters the quenching bath.

Similarly any wire of metal or alloy, which is annealed when quickly quenched from a relatively high temperature, may be treated by our method. Adjustment of voltage and speed in the heating zone will pass the wire into the liquid metal contact quench at the proper temperature for the particular material.

Before emerging from the quenching bath the wire will pick up the direct current supplied by the source 13 which is to effect the electrolytic pickling. Similar current will be supplied to the wire through the rinsing bath 10. By supplying the direct current to the wire in this manner substantially uniformity of current density is maintained in the wire within the pickling bath. From the wire 1 the current will flow through the pickling bath to the anode 12 and the desired electrolytic action is set up for the entire length of the anode 12.

From the pickling bath the treated wire is passed through a rinsing bath 10, which may preferably contain an agent which neutralizes the pickling bath which may be carried over in contact with the wire.

It will be observed that when conditioning chrome wire using our method and apparatus, selection may be made, in each step, of current having the characteristics which peculiarly adapt it to the work to be done. Also by using the quench bath and the rinse bath as contact means supplying current to the wire from one terminal of the electro-motive force used for electrolytic pickling, a highly desirable uniformity of current density in the wire is maintained in the portion which is being subjected to the pickling action.

Other forms may be employed embodying the features of our invention instead of the one explained, change being made as regards the means and the steps herein disclosed, provided the elements stated by any of the following claims or the equivalent of such stated elements be employed, whether produced by our preferred method or by others embodying steps equivalent to those stated in the following claims.

We therefore particularly point out and distinctly claim as our invention:

1. A method of conditioning in continuous operation a wire, or the like, formed of an alloy which softens and becomes more ductile when quickly quenched from a heated condition, comprising the steps of advancing such wire through an electrically conductive liquid bath; heating a section of such wire as it is advanced, by passing through such section a heating current of electricity supplied through such bath, which current is of strength sufficient to heat the wire to the desired temperature as it enters the bath; maintaining such bath at a desired temperature of quench; advancing such wire from the quench bath through a pickling bath; and passing through the liquid of the pickling bath, between an anode therein and the wire passing therethrough, a direct current of electricity from a source of electromotive force, one terminal of which is connected to such anode and the other terminal of which has electrical connection through such quench bath with the wire being treated.

2. A method of conditioning, in continuous operation, a wire, or the like, formed of an alloy which is annealed when quickly quenched from a heated condition, comprising the steps of advancing such wire through a bath of liquid metal; heating a section of such wire as it is advanced, by passing through such section a heating cur-

rent of electricity supplied through the metal bath, which current is of strength sufficient to heat the wire to the desired temperature as it enters the metal bath; maintaining the metal bath in a liquid condition at the desired quenching temperature; advancing such wire from the metal bath successively through a pickling bath and a rinsing bath; and passing through the liquid of the pickling bath, between an anode therein and the wire passing therethrough, a direct current of electricity from a source of electromotive force, one terminal of which is connected to such anode and the other terminal of which has electrical connections with such metal bath and with such rinsing bath.

3. Apparatus for conditioning in continuous operation a wire, or the like, formed of an alloy which anneals when quenched quickly from a heated condition, comprising in combination, an electrode; a quenching bath of liquid metal in spaced relation with said electrode; means maintaining a potential of electromotive force between said electrode and said bath; a bath of pickling solution; an anode extending longitudinally in said pickling bath; a bath of rinsing liquid; an electrical connection between said anode and the positive terminal of a source supplying a direct current of electricity; electrical connections between the negative terminal of said last-named source and said quenching bath and said rinsing bath; and means operative to advance a wire past said electrode in contact therewith and through said baths.

4. Apparatus for conditioning in continuous operation a wire, or the like, formed of an alloy, which anneals when quickly quenched from a heated condition, comprising in combination an electrode; a quenching bath of liquid metal in spaced relation with said electrode; means maintaining a potential of electromotive force between said electrode and said bath; a bath of pickling solution; an anode extending longitudinally in said pickling bath; an electrical connection between said anode and the positive terminal of a source supplying a direct current of electricity; an electrical connection between the negative terminal of said last-named source and said quenching bath; and means advancing a wire past said electrode in contact therewith and through said baths.

5. A method of conditioning, in continuous operation, a wire, or the like, formed of metallic material which softens and becomes more ductile when quenched from a critical temperature, comprising the steps of advancing such wire through a bath of quenching liquid; maintaining such bath at the desired quenching temperature; heating successive cross-sections of such wire by passing an electric current through a definite length thereof defined at its forward end by the surface of such quench bath; supplying current to such wire through such quench bath sufficient to raise the wire to the critical temperature as it enters the bath; advancing such wire from the quench bath to and through a bath of pickling liquid; and passing through the liquid of the pickling bath, between an anode therein and the wire passing therethrough, a direct current of electricity from a source of electromotive force, one terminal of which is electrically connected to such anode, and the other terminal of which has electrical connection with such quench bath.

6. Apparatus for conditioning in continuous operation a wire, or the like, comprising in combination, a quench bath of electrically conductive

- liquid maintained at a desired quenching temperature; means operative to heat a wire, continuously advanced into said bath, to a desired critical temperature in cross-sections thereof as they enter said bath, by its resistance to the passage of an electric current therethrough which current is supplied to such wire through said quench bath; a bath of pickling liquid; an anode extended longitudinally in said pickling bath; an electrically conductive connection between said anode and the positive terminal of a source supplying a direct current of electricity; an electrically conductive connection between the negative terminal of such source and the liquid of said quenching bath; and means operative to longitudinally advance a wire continuously through said baths.

7. Apparatus for conditioning in continuous operation a wire, or the like, comprising in combination a quenching bath of electrically conductive liquid maintained at a temperature desired for quenching a heated wire passed therethrough; a bath of pickling liquid; an anode extended longitudinally of said pickling bath; an electrically conductive connection between said anode and a terminal of a source of electromotive force; an electrically conductive connection between the liquid of said quench bath and the other terminal of such source; and means operative to longitudinally advance a heated wire into and through said quench bath and from it into and through said pickling bath. 15

WILLIAM H. WOOD.  
OSCAR C. TRAUTMAN.